



US011682509B2

(12) **United States Patent**  
**Chen et al.**

(10) **Patent No.:** **US 11,682,509 B2**  
(45) **Date of Patent:** **Jun. 20, 2023**

(54) **HIGH FREQUENCY MAGNETIC FILMS, METHOD OF MANUFACTURE, AND USES THEREOF**

(71) Applicant: **ROGERS CORPORATION**, Chandler, AZ (US)

(72) Inventors: **Yajie Chen**, Brighton, MA (US); **Xiaoyu Zhang**, Suzhou (CN); **Li Zhang**, Sichuan (CN); **Yuanyuan Xing**, Suzhou (CN)

(73) Assignee: **ROGERS CORPORATION**, Chandler, AZ (US)

(\*) Notice: Subject to any disclaimer, the term of this patent is extended or adjusted under 35 U.S.C. 154(b) by 863 days.

(21) Appl. No.: **16/676,736**

(22) Filed: **Nov. 7, 2019**

(65) **Prior Publication Data**

US 2020/0161034 A1 May 21, 2020

**Related U.S. Application Data**

(60) Provisional application No. 62/767,553, filed on Nov. 15, 2018.

(51) **Int. Cl.**

**H01F 1/16** (2006.01)  
**H01F 1/38** (2006.01)

(Continued)

(52) **U.S. Cl.**

CPC ..... **H01F 1/16** (2013.01); **H01F 1/38** (2013.01); **H01F 41/18** (2013.01); **H01F 41/32** (2013.01); **Y10T 428/32** (2015.01)

(58) **Field of Classification Search**

None

See application file for complete search history.

(56)

**References Cited**

U.S. PATENT DOCUMENTS

3,020,426 A 2/1962 Van Der Burgt  
3,036,007 A 5/1962 Buykx et al.

(Continued)

FOREIGN PATENT DOCUMENTS

CN 104356646 A 2/2015  
EP 620571 A2 \* 10/1994 ..... B82Y 25/00

(Continued)

OTHER PUBLICATIONS

Bid et al.; "Microstructure Characterization of Mechanothesized Nanocrystallizing NiFe<sub>2</sub>O<sub>4</sub> by Rietveld's Analysis"; Physica E 39; pp. 175-184; (2007).

(Continued)

*Primary Examiner* — Kevin M Bernatz

(74) *Attorney, Agent, or Firm* — Cantor Colburn LLP

(57)

**ABSTRACT**

A multilayer film includes a substrate; a first magnetic layer disposed on the substrate and a second magnetic layer disposed on the first magnetic layer. The first magnetic layer includes  $Fe_{(50-80)}N_{(10-20)}B_{(1-20)}M_{(0-10)}$ , wherein M is Si, Ta, Zr, Ti, Co, or a combination thereof. The second magnetic layer includes  $Fe_{(50-90)}N_{(10-50)}$  or  $Fe_{(60-90)}N_{(1-10)}Ta_{(5-30)}$ . The multilayer magnetic film has, over a frequency range of 50 MHz to 10 GHz, a magnetic permeability of greater than or equal to 1800 over a selected frequency band in the frequency range; a magnetic loss tangent of less than or equal to 0.3 over a selected frequency band in the frequency range; and a cutoff frequency of greater than or equal to 1 GHz, or greater than or equal to 2 GHz.

**13 Claims, 20 Drawing Sheets**



## (51) Int. Cl.

H01F 41/18 (2006.01)  
H01F 41/32 (2006.01)

## (56)

## References Cited

## U.S. PATENT DOCUMENTS

|                   |         |                      |                      |
|-------------------|---------|----------------------|----------------------|
| 5,591,276 A *     | 1/1997  | Yoshizawa .....      | C22C 45/02<br>420/83 |
| 6,071,430 A       | 6/2000  | Lebourggeois et al.  |                      |
| 6,436,307 B1      | 8/2002  | Lebourggeois et al.  |                      |
| 6,736,990 B2      | 5/2004  | Aoki et al.          |                      |
| 7,348,374 B2      | 3/2008  | Martinazzo           |                      |
| 7,482,977 B2      | 1/2009  | Kuroda et al.        |                      |
| 10,071,421 B2     | 9/2018  | Suetsuna et al.      |                      |
| 10,090,088 B2     | 10/2018 | Suetsuna et al.      |                      |
| 2003/0091841 A1   | 5/2003  | Marusawa             |                      |
| 2004/0069969 A1   | 4/2004  | Endo et al.          |                      |
| 2007/0231614 A1   | 10/2007 | Kondo et al.         |                      |
| 2009/0057606 A1   | 3/2009  | Tada et al.          |                      |
| 2010/0151797 A1 * | 6/2010  | Viala .....          | H01F 41/32<br>455/73 |
| 2011/0147643 A1   | 6/2011  | Ryou et al.          |                      |
| 2012/0068103 A1   | 3/2012  | Hill et al.          |                      |
| 2012/0229354 A1   | 9/2012  | Ishikura et al.      |                      |
| 2014/0291571 A1   | 10/2014 | Hirose               |                      |
| 2014/0346387 A1   | 11/2014 | Hill et al.          |                      |
| 2016/0086700 A1   | 3/2016  | Suetsuna et al.      |                      |
| 2016/0086728 A1   | 3/2016  | Suetsuna et al.      |                      |
| 2016/0099498 A1   | 4/2016  | Pance et al.         |                      |
| 2016/0113113 A1   | 4/2016  | Sethumadhavan et al. |                      |
| 2016/0276072 A1   | 9/2016  | Sethumadhavan et al. |                      |
| 2017/0098885 A1   | 4/2017  | Hill et al.          |                      |
| 2019/0081377 A1   | 3/2019  | Hill et al.          |                      |
| 2021/0020343 A1   | 1/2021  | Chen et al.          |                      |

## FOREIGN PATENT DOCUMENTS

|    |               |         |
|----|---------------|---------|
| EP | 0620571 A2    | 10/1994 |
| EP | 1541641 A1    | 6/2005  |
| EP | 1652829 A2    | 5/2006  |
| JP | H01200605 A   | 8/1989  |
| JP | 2001085210 A  | 3/2001  |
| WO | 2017068444    | 4/2017  |
| WO | 2018043943 A1 | 3/2018  |

## OTHER PUBLICATIONS

Chicinas, I.; "Soft Magnetic Nanocrystalline Powders Produced by Mechanical Alloying Routes"; Journal of Optoelectronics and Advanced Materials; 8(2); pp. 439-448; (2006).

International Search Report; International Application No. PCT/US2019/060229; International Filing Date: Nov. 7, 2019; dated Mar. 13, 2020; 7 pages.

Ismail et al.; "Magnetic Properties of Mechanically Alloyed Cobalt-Zinc Ferrite Nanoparticles"; J. Supercond Nov Magn; 27; pp. 1293-1298; (2014).

Koch, C. C.; "Materials Synthesis by Mechanical Alloying"; Annu. Rev. MaterSci. 19; pp. 121-143; (1989).

Koch, C. C.; "Intermetallic Matrix Composites Prepared by Mechanical Alloying—a Review"; Materials Science and Engineering; A244; pp. 39-48; (1998).

Kong et al., "Ni—Zn Ferrites Composites With Almost Equal Values of Permeability and Permittivity for Low-Frequency Antenna Design," IEEE Transactions on Magnetics, Jan. 2007, pp. 6-9, vol. 43, No. 1.

Ohnuma et al., "Soft Magnetic Properties of FeN/FeBN Multilayers," Journal on Magnetics, Nov. 1992, pp. 896-901, vol. 7 No. 11.

Ohnuma et al., "Soft Magnetic Multilayers for Micromagnetic Devices," Journal of Magnetism and Magnetic Materials, 1993, pp. 556-562, vol. 126.

Sepelak et al.; "Nanocrystalline Nickel Ferrite, NiFe<sub>2</sub>O<sub>4</sub>: Mechanosynthesis, Nonequilibrium Cation Distribution, Canted Spin Arrangement, and Magnetic Behavior"; J.Phys.Chem. C; 111; pp. 5026-5033; (2007).

Sepelak et al.; "Structural and Magnetic Properties of Nanosize Mechanothesized Nickel Ferrite"; Journal of Magnetism and Magnetic Materials; 272-276; pp. 1616-1618; (2004).

Waje et al.; "Sintering Temperature dependence of Room Temperature Magnetic and Dielectric Properties of Co<sub>0.5</sub>Zn<sub>0.5</sub>F<sub>3</sub>O<sub>4</sub> Prepared using Mechanically Alloyed Nanoparticles"; Journal of magnetism and Magnetic Materials; 322; pp. 686-691; (2010).

Written Opinion; International Application No. PCT/US2019/060229; International Filing Date: Nov. 7, 2019; dated Mar. 13, 2020; 8 pages.

Martin et al.; "Flexible Magnetic Composites"; Passive RF Component Technoloby, Materials Techniques and Applications; Chapter 8; 2012; pp. 156-185.

Thakur et al.; "Low-loss Spinel Nanoferrite With Matching Permeability and Permittivity in the Ultrahigh Frequency Range"; Journal of Applied Physics; 108, 014301; (2010).

Yang, Guo-Min, et al., "Miniaturized Patch Antennas with Ferrite/Dielectric/Ferrite Magnetodielectric Sandwich Substrate", Piers Online, vol. 7, No. 7, (Jan. 1, 2011), pp. 609-612.

Pullar, "Hexagonal Ferrites: A Review of the synthesis, properties and application of hexaferrite ceramics," Mar. 2012, Progress in Material Science, vol. 57, No. 7, pp. 1191-1334.

Raja et al., "1.12: An Introduction to Energy Dispersive X-ray Spectroscopy", p. 80-84, from "Physical Methods in Chemistry and Nano Science", LibreText,Text Compiled on Dec. 5, 2022; 693 pages.

\* cited by examiner



Fig. 1



Fig. 2



Fig. 3



*Fig. 4*



*Fig. 5*



Fig. 6



Fig. 7



Fig. 8



Fig. 9



Fig. 10



Fig. 11



Fig. 12



Fig. 13



Fig. 14



Fig. 15



Fig. 16



Fig. 17



*Fig. 18*



Fig. 19



Fig. 20



Fig. 21



Fig. 22



Fig. 23



Fig. 24



Fig. 25



Fig. 26



Fig. 27



Fig. 28

**HIGH FREQUENCY MAGNETIC FILMS,  
METHOD OF MANUFACTURE, AND USES  
THEREOF**

**CROSS REFERENCE TO RELATED  
APPLICATION**

This application claims the benefit of U.S. Provisional Patent Application Ser. No. 62/767,553 filed Nov. 15, 2018. The related application is incorporated herein in its entirety by reference.

**BACKGROUND**

This disclosure relates generally to high frequency magnetic films, methods for their manufacture, and uses thereof, for example in integrated circuits, power supply systems, antennas, and the like.

Newer designs and manufacturing techniques have driven electronic components to increasingly smaller dimensions and higher frequencies. One approach to reducing electronic component size has been the use of magnetic materials. In particular, ferrites, ferroelectrics, and multiferroics have been widely studied as functional materials with enhanced microwave properties. While the high permeability of magnetic materials increases the DC value of inductance, it remains a challenge to extend that magnetic permeability and corresponding inductance enhancement to high frequencies (e.g., 1 to 5 gigahertz (GHz)), which are desired for various mobile applications. Magnetic permeability at these frequencies is sharply deteriorated due to Snoek's limit of the materials. At the intrinsic ferromagnetic resonance (FMR) frequency of magnetic materials (typically 1-2 GHz for large blanket films), the relative magnetic permeability drops to unity and the magnetic loss tangent peaks, such that the inductance enhancement due to the material is negligible and the losses are dominant. It is possible to enhance the frequency response of magnetic permeability by varying methods of definition and patterning of the materials, but there still remains a need in the art for materials and methods that can provide high magnetic permeability and high resonance frequency over high bandwidths.

**BRIEF DESCRIPTION**

Disclosed herein is a multi-layer magnetic film and a method of making the same.

In an embodiment, a multilayer film includes a substrate; a first magnetic layer disposed on the substrate and a second magnetic layer disposed on the first magnetic layer. The first magnetic layer includes  $Fe_{(50-80)}N_{(10-20)}B_{(1-20)}M_{(0-10)}$ , wherein M is Si, Ta, Zr, Ti, Co, or a combination thereof. The second magnetic layer includes  $Fe_{(50-80)}N_{(10-20)}B_{(1-20)}M_{(0-10)}$ . The multilayer magnetic film has, over a frequency range of 50 megahertz (MHz) to 10 GHz, preferably over a frequency range of 100 MHz to 5 GHz, more preferably over a frequency range of 1 to 5 GHz, a magnetic permeability of greater than or equal to 1800, preferably greater than or equal to 2000, more preferably greater than or equal to 3000 to 5000 over a selected frequency band in the frequency range, preferably over a frequency band of 1 to 10 GHz; a magnetic loss tangent of less than or equal to 0.3, preferably less than or equal to 0.1, more preferably 0.01 to 0.1 over a selected frequency band in the frequency range, preferably over a frequency band of 1 to 10 GHz; and a cutoff

frequency of greater than or equal to 1 GHz, or greater than or equal to 2 GHz, preferably greater than or equal to 5 GHz, or 1 to 8 GHz.

In an embodiment, a method of forming the multilayer film includes depositing the first magnetic layer onto a side of the substrate; and depositing the second magnetic layer onto a side of the first magnetic layer opposite to the substrate.

Articles includes the multi-layer magnetic films are further described. The article is preferably a filter, transformer, inductor, antenna, electronic integrated circuit chip, or electromagnetic shielding device.

The above and other features and advantages are readily apparent from the following detailed description, examples, and claims when taken in connection with the accompanying drawings.

**BRIEF DESCRIPTION OF THE DRAWINGS**

20 Referring to the exemplary non-limiting figures wherein like elements are numbered alike:

FIG. 1 is a cross-sectional view of an embodiment of a multilayer magnetic film;

FIG. 2 is a cross-sectional view of another embodiment of a multilayer magnetic film;

FIG. 3 is a plot showing the high frequency characteristics of comparative Co- and Fe-based thin films and multilayers measured at room temperature;

FIG. 4 is a surface profile of an FeN film by profilometry and atomic force microscopy (AFM);

FIG. 5 is a magnetic hysteresis of FeN films along easy and hard magnetizing directions in a plane of the film;

FIG. 6 is a magnetic permeability spectrum of an FeN film with 60 nanometer (nm) thickness;

35 FIG. 7 is a surface profile of an FeN film by profilometry and AFM;

FIG. 8 is a magnetic permeability spectrum of an  $Fe_{66}N_{18}B_{16}$  film with 50 nm thickness;

FIG. 9 shows the relationship between effective resistivity and magnetic permeability of an  $Fe_{83-x}N_{17}B_x$  film with differing boron content;

FIG. 10 is magnetic spectra of  $Fe_{74}N_{26}/Fe_{66}N_{18}B_{16}$  bi-layer films with various thicknesses of FeNB;

45 FIG. 11 is a magnetic permeability for  $Fe_{74}N_{26}/Fe_{72}N_{18}B_{10}$  bi-layer films with different thicknesses of  $Fe_{72}N_{18}B_{10}$ ;

FIG. 12 shows the relationship between effective resistivity and magnetic permeability of an  $Fe_{82}N_{18}/Fe_{72}N_{18}B_{10}$ /glass film with different thicknesses of an FeNB layer;

50 FIG. 13 is a magnetic hysteresis of an FeTaN film with thickness of 80 nm along x and y directions in a plane of the film;

FIG. 14 is a magnetic permeability spectrum of 80 nm-thick  $Fe_{74}Ta_6N_{20}$  film on a glass substrate;

55 FIG. 15 is magnetic spectra for  $Fe_{74}Ta_6N_{20}/Fe_{66}N_{18}B_{16}$  bi-layer films;

FIG. 16 shows the relationship between effective resistivity and magnetic permeability of an  $Fe_{83}Ta_6N_{11}/Fe_{72}N_{18}B_{10}$ /glass film with different thicknesses of an FeNB layer;

60 FIG. 17 is magnetic spectra for  $Fe_{74}Ta_6N_{20}/Fe_{72}N_{18}B_{10}$  bi-layer films;

FIG. 18 shows the relationship between effective resistivity and total tri-layer film thickness of  $Fe_{72}N_{18}B_{10}/Fe_{83}N_{11}/Fe_{72}N_{18}B_{10}$  tri-layer films;

65 FIG. 19 is magnetic spectra of  $Fe_{72}N_{18}B_{10}/Fe_{82}N_{18}/Fe_{82}N_{18}B_{10}$  tri-layer films;

FIG. 20 shows the relationship between effective resistivity and total tri-layer film thickness of an  $\text{Fe}_{72}\text{N}_{18}\text{B}_{10}/\text{Fe}_{83}\text{Ta}_6\text{N}_{18}/\text{Fe}_{72}\text{N}_{18}\text{B}_{10}$  tri-layered structure;

FIG. 21 is magnetic spectra of an  $\text{Fe}_{72}\text{N}_{18}\text{B}_{10}/\text{Fe}_{72}\text{Ta}_{18}\text{N}_{10}/\text{Fe}_{72}\text{N}_{18}\text{B}_{10}$  tri-layered structure;

FIG. 22 is magnetic spectra for  $\text{Fe}_{82}\text{N}_{18}/\text{Ta}_{88}\text{N}_{12}$  bilayer films;

FIG. 23 is magnetic spectra for  $\text{Fe}_{72}\text{N}_{18}\text{B}_{10}/\text{Ta}_{88}\text{N}_{12}$  bilayer films;

FIG. 24 is magnetic spectra for  $\text{Fe}_{83}\text{Ta}_6\text{N}_{11}/\text{Ta}_{88}\text{N}_{12}$  bilayer films;

FIG. 25 shows magnetic permeability at 0.5 GHz for a single layer, bi-layer and tri-layer FeN-based films;

FIG. 26 is a Snoek product diagram at 0.5 GHz for a single layer, bi-layer and tri-layer FeN-based multi-layered structure;

FIG. 27 shows magnetic permeability at 0.5 GHz for a single layer, bi-layer and tri-layer FeTaN-based multi-layered structure; and

FIG. 28 is a Snoek product diagram at 0.5 GHz for a single layer, bi-layer and tri-layer FeTaN-based multi-layered structure.

#### DETAILED DESCRIPTION

The inventors hereof have developed multilayer magnetic films with a combination of high magnetic permeability, low loss, and excellent inductance over a broad frequency range. The magnetic thin-films integrated with complementary metal-oxide-semiconductor (CMOS) enable high-quality, high density, low-profile, on-chip/in-package inductive components.

The multilayer films are disposed on a substrate, and include a first magnetic layer, wherein the first magnetic layer comprises  $\text{Fe}_{(50-80)}\text{N}_{(10-20)}\text{B}_{(1-20)}\text{M}_{(0-10)}$ , wherein M is Si, Ta, Zr, Ti, Co, Nb, or a combination thereof (herein referred to as FeNB); and a second magnetic layer wherein the second magnetic layer comprises  $\text{Fe}_{(50-90)}\text{N}_{(10-50)}$  (herein referred to as FeN) or  $\text{Fe}_{(60-90)}\text{N}_{(1-10)}\text{Ta}_{(5-30)}$  (herein referred to as FeNTa). The multilayer magnetic films can operate over a frequency range of 50 MHz to 10 GHz and can have a magnetic constant (also known as a magnetic permeability) of greater than or equal to 1800 and a magnetic loss tangent of less than or equal to 0.3 measured over a selected frequency band.

An illustration of a cross-sectional view of a multilayer magnetic film 10 is shown in FIG. 1. Substrate 12 has a first side, i.e., a first planar surface and a second side, i.e., an opposite second planar surface. The substrate 12 can be of any suitable material, for example a glass, an organic polymer, or a ceramic. In an aspect, the substrate comprises a ceramic such as at least one of MgO, Sic,  $\text{Si}_3\text{N}_4$ , alumina, silicon, or the like. The substrate can be amorphous, single crystal, or polycrystalline. The substrate 12 can have any suitable thickness, which will depend on its support properties and the intended application. For example, the substrate can have a thickness of 100 micrometers to 1 millimeters.

The first magnetic layer 14 is disposed on the first side of the first planar surface. As stated above, the first magnetic layer comprises  $\text{Fe}_{(50-80)}\text{N}_{(10-10)}\text{B}_{(1-20)}\text{M}_{(0-10)}$ , wherein M is Si, Ta, Zr, Ti, Co, Nb, or a combination thereof. In a preferred aspect, the first magnetic layer comprises  $\text{Fe}_{(50-80)}\text{N}_{(10-20)}\text{B}_{(1-20)}$ , wherein the amount of M is 0. The first magnetic layer can have a thickness of 10 to 100 nanometers, for example 10 to 50 nanometers or 20 to 80 nanometers.

A second magnetic layer 16 is disposed on a side of the first magnetic layer opposite the substrate. The second magnetic layer comprises  $\text{Fe}_{(50-90)}\text{N}_{(10-50)}$  or  $\text{Fe}_{(60-90)}\text{N}_{(1-10)}\text{Ta}_{(5-30)}$ . The second magnetic layer can have a thickness of 10 to 400 nanometers, for example 10 to 300 nanometers, or 50 to 400 nanometers.

The multilayer magnetic film can include additional layers, in particular additional alternating first and second layers. As shown in FIG. 2, an additional first magnetic layer 16, comprising  $\text{Fe}_{(50-80)}\text{N}_{(10-20)}\text{B}_{(1-20)}$ , is disposed on the second magnetic layer 14. An additional second magnetic layer 18, comprising  $\text{Fe}_{(50-90)}\text{N}_{(10-50)}$  or  $\text{Fe}_{(60-90)}\text{N}_{(1-10)}\text{Ta}_{(5-30)}$ , is disposed on the additional first magnetic layer 16. Further additional first and second magnetic layers can be disposed on the additional second magnetic layer in alternation (not shown).

The first magnetic layer 14 and the second magnetic layer 16 can have a total thickness of 20 to 500 nanometers. In an embodiment the first magnetic layer 14 has a thickness of 10 to 200 nm, and the second magnetic layer can have a thickness of 10 to 400 nm. In a particularly advantageous feature, the thickness of each of the magnetic layers, the ratio of the thickness, or both, can be adjusted to obtain a desired magnetic loss tangent of the multilayer magnetic film, a desired magnetic anisotropy of the magnetic multilayer film, or both.

A method of forming the multilayer magnetic film includes depositing the first magnetic layer onto a side of the substrate; and depositing the second magnetic layer onto a side of the first magnetic layer opposite to the substrate. Deposition of alternating layers proceeds until the entire film is manufactured. Deposition can be by rf/DC sputtering, electron beam deposition, or a combination thereof.

The multilayer magnetic films can be used over a frequency range of 50 MHz to 10 GHz, preferably over a frequency range of 100 MHz to 5 GHz, more preferably over a frequency range of 1 to 5 GHz.

The multilayer magnetic films can have a magnetic permeability of greater than or equal to 1800, preferably greater than or equal to 2000, more preferably greater than or equal to 3000, or 1800 to 5000 over a selected frequency band in the frequency range, preferably over a frequency band of 1 to 10 GHz. As used herein, this terminology refers to the multilayer magnetic films having at least one instance of the magnetic permeability being greater than or equal to 1800 over the frequency band of 1 to 5 GHz, or 1 to 10 GHz.

The multilayer magnetic films can have a magnetic loss tangent of less than or equal to 0.3, or less than 0.3, preferably less than or equal to 0.1, or less than 0.1, or 0.01 to 0.3 over a selected frequency band in the frequency range, preferably over a frequency band of 1 to 10 GHz. As used herein, this terminology refers to the multilayer magnetic films having at least one instance of the magnetic loss tangent being less than or equal to 0.3 over the frequency band of 1 to 5 GHz, or 1 to 10 GHz.

The multilayer magnetic films can have a cutoff frequency of greater than or equal to 1 GHz, or greater than 1 GHz, or greater than or equal to 2 GHz, preferably greater than or equal to 5 GHz, or 1 to 8 GHz.

The multilayer magnetic films can include additional layers, for example, a top layer. The top layer can include  $\text{Al}_2\text{O}_3$ . The top layer can include an insulating cap.

The multilayer magnetic films can be used in electronic devices such as filters or inductors on electronic integrated circuit chips for a wide variety of applications, for example, electric power applications, data storage, and microwave communication. The multilayer magnetic film can be used in

low frequency applications, for example, at a frequency of 50 MHz to 1 GHz, or in high frequency applications, for example 1 to 10 GHz. The multilayer magnetic film can be used in antennas, and in electronic devices such as mobile internet devices, and in electronic devices, for example, cell phones, tablets, desktop computers, laptop computers, note-

the 60 nm thick FeN film on glass substrate is provided in Table 1. In FIGS. 5 and 13, Easy (solid lines) or Hard (dashed lines) magnetizing direction indicates an energetically favorable or unfavorable direction of spontaneous magnetization, respectively.

TABLE 1

| Film thickness<br>(nm) | 0.5 GHz |              | 1 GHz |              | 1.5 GHz |              | $f_r$<br>(GHz) | Snoek product<br>( $\times 10^{12}$ ) | 4πMs<br>(kG) | Hc<br>(Oe) |
|------------------------|---------|--------------|-------|--------------|---------|--------------|----------------|---------------------------------------|--------------|------------|
|                        | $\mu'$  | $\tan\delta$ | $u'$  | $\tan\delta$ | $u'$    | $\tan\delta$ |                |                                       |              |            |
| 60                     | 510     | 0.31         | 539   | 0.22         | 788     | 0.84         | 1.71           | 0.87                                  | 12.43        | 1.9        |

book computers, and the like. In an aspect, the device is a portable electronic device, for example a handheld electronic device. The multilayer magnetic films can further be used in power supply systems and antennas. The multilayer magnetic films can advantageously be used in integrated electronic devices.

The following examples are provided to illustrate the present disclosure. The examples are merely illustrative and are not intended to limit devices made in accordance with the disclosure to the materials, conditions, or process parameters set forth therein.

### EXAMPLES

FIG. 3 is a plot showing initial magnetic permeability versus resonance frequency/gigahertz (GHz) of various comparative films, reproduced from Chin. Phys. B Vol. 24, No. 5 (2015) 05750.

#### Example 1: FeN/FeNB/Glass Bi-Layered Film Structure

##### Parameters for RF Magnetron Sputtering:

RF Power=80 to 120 Watts (W)

Deposition pressure=0.3 to 0.6 pascals (Pa)

Distance between target and substrate=8 centimeters (cm)

Working gas: Argon; Reaction gas: Nitrogen

Target:

Iron (99.9%), 2-inch (5.08 cm) disk;

2 pieces of boron (99.9%) chip with 2.5×2.5 square millimeters ( $\text{mm}^2$ )

Deposition time: 5 to 30 minutes

Deposition temperature: ambient

Substrate: Optical glass

##### Single Layer of FeN Film on Glass Substrate (Reference Example)

With reference to FIGS. 4-6, an FeN film had a composition of  $\text{Fe}_{74}\text{N}_{26}$  and thickness of 60 nanometers (nm) on a glass substrate, measured by (energy-dispersive X-ray spectroscopy) EDXS and profilometry, respectively. EDXS provides elemental analysis of the composition, and as such it will be understood that the subscripts in the Formula (i.e.,  $\text{Fe}_{74}\text{N}_{26}$ ) refer to the atomic ratio of each element (i.e., Fe to N). In the figures, the abbreviation G1 stands for glass. The FeN film having a film thickness of 60 nm exhibited a fine grain size of 11 nm by atomic force microscopy (AFM). The FeN film exhibited magnetic anisotropy in the film plane depicted in magnetic hysteresis loops. The FeN film had a magnetic permeability ( $\mu'$ ) of 510 at 0.5 gigahertz (GHz) and a magnetic loss tangent ( $\tan\delta$ ) of 0.3 and retained a resonance frequency of 1.71 GHz. The FeN film had a Snoek product of  $0.87 \times 10^{12}$ . A summary of magnetic properties for

##### 15 Single Layer of FeNB Film on Glass Substrate (Reference Example)

With reference to FIGS. 7 and 8, the FeNB film on a glass substrate had a composition of  $\text{Fe}_{66}\text{N}_{18}\text{B}_{16}$  and thickness of 50 nm and an average grain size of 6.7 nm, measured by EDXS and profilometry, respectively. The FeNB film on a glass exhibited a magnetic permeability of 864 at 1 GHz and Snoek product of  $1.26 \times 10^{12}$ , respectively. A summary of magnetic measurements for the  $\text{Fe}_{66}\text{N}_{18}\text{B}_{16}$  film is provided in Table 2.

TABLE 2

| Film thickness<br>(nm) | 0.5 GHz |              | 1 GHz |              | 1.5 GHz |              | $f_r$<br>(GHz) | Snoek product<br>( $\times 10^{12}$ ) | 4πMs<br>(kG) | Hc<br>(Oe) |
|------------------------|---------|--------------|-------|--------------|---------|--------------|----------------|---------------------------------------|--------------|------------|
|                        | $\mu'$  | $\tan\delta$ | $u'$  | $\tan\delta$ | $u'$    | $\tan\delta$ |                |                                       |              |            |
| 50                     | 730     | 0.19         | 864   | 0.18         | 1547    | 0.80         | 1.73           | 1.26                                  | 1.26         | 1.26       |

35 With reference to FIG. 9, the effective resistivity of the FeNB film increased with an increase in the content of boron ( $x=0, 13, 14, 16, 19$ ). The magnetic permeability at 0.5 GHz was increased in the resistivity range from 400 to 450 microohm meters ( $\mu\Omega\text{m}$ ).

##### 40 FeN/FeNB Bi-Layer on a Glass Substrate

An  $\text{Fe}_{66}\text{N}_{18}\text{B}_{16}$  film was deposited onto a glass substrate, followed by deposition of an  $\text{Fe}_{74}\text{N}_{26}$  film with a constant thickness of 50 nm. The thickness of the  $\text{Fe}_{66}\text{N}_{18}\text{B}_{16}$  film was in a range of 10-35 nm, varying with deposition time. FIG. 10 shows  $\mu'$  (solid lines) and  $\mu''$  (dashed lines) for varying thicknesses of the  $\text{Fe}_{66}\text{N}_{18}\text{B}_{16}$  film in nm as indicated on the figure.

With reference to FIG. 10, an FeN (50 nm)/FeNB (23 nm) bi-layer film exhibited a high magnetic permeability of 1832 at 0.5 GHz and Snoek product of  $3.72 \times 10^{12}$ , respectively. The FeN (50 nm)/FeNB (23 nm) bi-layer film exhibited high magnetic permeability of 2313 at 1.5 GHz. The composition of the FeNB film was measured to be  $\text{Fe}_{66}\text{N}_{18}\text{B}_{16}$  by EDXS.

55 A summary of magnetic measurements for the FeN/FeNB bi-layered films with different thicknesses of the FeNB layer is provided in Table 3.

TABLE 3

| Film thickness<br>(nm) | 0.5 GHz |              | 1 GHz |              | 1.5 GHz |              | $f_r$<br>(GHz) | Snoek product<br>( $\times 10^{12}$ ) | 4πMs<br>(kG) | Hc<br>(Oe) |
|------------------------|---------|--------------|-------|--------------|---------|--------------|----------------|---------------------------------------|--------------|------------|
|                        | $\mu'$  | $\tan\delta$ | $u'$  | $\tan\delta$ | $u'$    | $\tan\delta$ |                |                                       |              |            |
| 10                     | 899     | 0.44         | 1103  | 0.44         | 853     | 1.98         | 1.62           | 1.46                                  | 1.46         | 1.46       |
| 20                     | 1062    | 0.53         | 1366  | 0.30         | 3221    | 0.41         | 1.83           | 1.94                                  | 1.94         | 1.94       |
| 23                     | 1832    | 0.21         | 1679  | 0.27         | 2313    | 0.33         | 2.03           | 3.72                                  | 3.72         | 3.72       |

TABLE 3-continued

| Film thickness (nm) | 0.5 GHz |              | 1 GHz |              | 1.5 GHz |              | $f_r$ (GHz) | Snoek product ( $\times 10^{12}$ ) |
|---------------------|---------|--------------|-------|--------------|---------|--------------|-------------|------------------------------------|
|                     | $\mu'$  | $\tan\delta$ | $u'$  | $\tan\delta$ | $u'$    | $\tan\delta$ |             |                                    |
| 30                  | 1042    | 0.02         | 1275  | 0.01         | 2069    | 0.29         | 2.01        | 2.09                               |
| 35                  | 853     | 0.09         | 1375  | 0.01         | 2201    | 0.23         | 2.01        | 1.71                               |

Example 2: FeN/FeNB/Glass Bi-Layered Film Structure with Low Level of Boron Content

Parameters for RF Magnetron Sputtering:

RF Power=80 to 120 W

Deposition pressure=0.3 to 0.6 pascals (Pa)

Distance between target and substrate=8 centimeters (cm)

Working gas: Ar; Reaction gas: Nitrogen

Target:

Iron (99.5%), 2-inch disk

2 pieces of boron (99.5%) chip with  $2.5 \times 2.5 \text{ mm}^2$

Deposition time: 5 to 30 minutes

Deposition temperature: ambient

Substrate: Optical glass

In this example, an FeNB film was deposited onto a glass substrate, followed by a 50 nm thick FeN film deposited on the top of the FeNB film at ambient temperature. The thickness of the FeNB film varied with deposition time, and a constant thickness of 50 nm for the FeN film was retained. Magnetic Permeability Spectra for FeN/FeNB Films with Low Level of Boron Content

With reference to FIG. 11, the FeNB film had a composition of  $\text{Fe}_{72}\text{N}_{18}\text{B}_{10}$ , and the FeN had a composition of  $\text{Fe}_{74}\text{N}_{26}$  measured by EDXS. FIG. 11 shows (solid lines) and  $\mu''$  (dashed lines) for varying thicknesses of the  $\text{Fe}_{66}\text{N}_{18}\text{B}_{10}$  film in nm as indicated on the figure. The bi-layered film structure exhibited an increased magnetic permeability from 1207 to 1741 with an increased thickness of the FeNB seed layer from 15 nm to 25 nm. The Snoek product of the FeN/FeNB film increased by 60% with an increase of thickness of the FeNB seed layer from 15 nm to 25 nm. A summary of magnetic spectrum measurements for the  $\text{Fe}_{74}\text{N}_{26}/\text{Fe}_{72}\text{N}_{18}\text{B}_{10}$  bi-layer films is provided in Table 4.

TABLE 4

| FeNB thickness in FeN (50 nm)/FeNB/Glass (nm) | 0.5 GHz |              | 1 GHz |              | 1.5 GHz |              | $f_r$ (GHz) | Snoek product ( $\times 10^{12}$ ) |
|-----------------------------------------------|---------|--------------|-------|--------------|---------|--------------|-------------|------------------------------------|
|                                               | $\mu'$  | $\tan\delta$ | $u'$  | $\tan\delta$ | $u'$    | $\tan\delta$ |             |                                    |
| 15                                            | 895     | 0.08         | 1207  | 0.04         | 2023    | 0.31         | 2.08        | 1.86                               |
| 20                                            | 1248    | 0.18         | 1707  | 0.15         | 2951    | 0.58         | 1.81        | 2.26                               |
| 22                                            | 1427    | 0.11         | 1599  | 0.05         | 2690    | 0.45         | 1.96        | 2.80                               |
| 25                                            | 1561    | 0.18         | 1741  | 0.06         | 3094    | 0.27         | 1.91        | 2.98                               |
| 30                                            | 1297    | 0.16         | 1657  | 0.13         | 2972    | 0.38         | 1.91        | 2.48                               |

Resistivity Versus Magnetic Permeability (at 0.5 GHz) for a FeN/FeNB/Glass Structure

With reference to FIG. 12, the effective resistivity of the FeN/FeNB/Glass film was affected by the thickness of the FeNB seed layer. The resistivity increased with an increase of the FeNB thickness. Magnetic permeability at 0.5 GHz was increased in the resistivity range from 460 to 490  $\mu\Omega\text{m}$ .

Example 3: FeTaN/FeNB/Glass Bi-Layered Structure Parameters for RF Magnetron Sputtering

RF Power=80 to 120 W

Deposition pressure=0.3 to 0.6 pascals (Pa)

Distance between target and substrate=8 centimeters (cm)

Working gas: Ar (99.5%); Reaction gas: Nitrogen (99.0%)

Target:

Iron (99.5%), 2-inch disk

2 pieces of boron (99.5%) chip with  $5 \times 5 \text{ mm}^2$

Deposition time: 5 to 30 minutes

Deposition temperature: ambient

Substrate: Optical glass

Magnetic Properties and Magnetic Permeability of Single FeTaN Film on a Glass Substrate

With reference to FIGS. 13 and 14, a summary of magnetic spectrum measurements for a  $\text{Fe}_{74}\text{TaN}_{20}$  single film is provided in Table 5.

TABLE 5

| Film thickness (nm) | 0.5 GHz |              | 1 GHz |              | 1.5 GHz |              | $f_r$ (GHz) | Snoek product ( $\times 10^{12}$ ) | $4\pi M_s$ (kG) | $H_c$ (Oe) |
|---------------------|---------|--------------|-------|--------------|---------|--------------|-------------|------------------------------------|-----------------|------------|
|                     | $\mu'$  | $\tan\delta$ | $u'$  | $\tan\delta$ | $u'$    | $\tan\delta$ |             |                                    |                 |            |
| 80                  | 539     | 0.85         | 752   | 0.41         | 876     | 1.78         | 1.63        | 0.88                               | 12.9            | 1.88       |

Magnetic Permeability of Bi-Layered FeTaN/FeNB Films on the Glass Substrate

With reference to FIG. 15, the bi-layered film structure included  $Fe_{74}Ta_6N_{20}$  and  $Fe_{66}N_{18}B_{16}$  films deposited on a glass substrate. A summary of magnetic spectrum measurements for  $Fe_{74}Ta_6N_{20}/Fe_{66}N_{18}B_{16}$  bilayer films is provided in Table 6.

TABLE 6

| FeNB thickness in FeTaN(50 nm)/FeNB/Glass (nm) | 0.5 GHz |              | 1 GHz  |              | 1.5 GHz |              | $f_r$ | Snoek product ( $\times 10^{12}$ ) |
|------------------------------------------------|---------|--------------|--------|--------------|---------|--------------|-------|------------------------------------|
|                                                | $\mu'$  | $\tan\delta$ | $\mu'$ | $\tan\delta$ | $\mu'$  | $\tan\delta$ | (GHz) |                                    |
| 15                                             | 913     | 0.10         | 814    | 0.14         | 1621    | 0.55         | 1.70  | 1.55                               |
| 20                                             | 1167    | 0.03         | 953    | 0.24         | 1882    | 0.78         | 1.61  | 1.88                               |
| 22                                             | 1130    | 0.11         | 1168   | 0.13         | 2044    | 1.02         | 1.88  | 1.88                               |

Resistivity Versus Magnetic Permeability (at 0.5 GHz) for a FeTaN/FeNB/Glass Structure

With reference to FIG. 16, the effective resistivity of the FeNB/FeTaN film was affected by the thickness of the FeNB layer. The effective resistivity increased from 438  $\mu\Omega m$  to 489  $\mu\Omega m$  with an increase of the FeNB thickness from 60 nm to 75 nm. High magnetic permeability was exhibited in a resistivity range from 430 to 460  $\mu\Omega m$ .

Example 4: FeTaN/FeNB/Glass Bi-Layer Film Structure with Low Level of Boron Content Parameters for RF Magnetron Sputtering

RF Power=80 to 120 W

Deposition pressure=0.3 to 0.6 pascals (Pa)

Distance between target and substrate=8 centimeters (cm)

Working gas: Ar (99.5%); Reaction gas: Nitrogen (99.0%)

Target:

Iron (99.5%), 2-inch disk

2 pieces of boron (99.5%) chip with  $5 \times 5 \text{ mm}^2$

1 piece for tantalum (99.99%) ( $5 \times 5 \text{ mm}^2$ )

Deposition time: 5 to 30 minutes

Deposition temperature: ambient

Substrate: Optical glass

Magnetic Permeability Spectrum of in FeTaN/FeNB Film with Low Level of B Concentration

With reference to FIG. 17, the FeTaN film had a composition of  $Fe_{74}Ta_6N_{20}$  measured by EDXS, and FeNB had a composition of  $Fe_{72}N_{18}B_{10}$ . FIG. 17 shows  $\mu'$  (solid lines) and  $\mu''$  (dashed lines) for varying thicknesses of the  $Fe_{72}N_{18}B_{10}$  film in nm as indicated on the figure. A summary of magnetic spectrum measurements for  $Fe_{74}Ta_6N_{20}/Fe_{72}N_{18}B_{10}$  bilayer films on a glass substrate is provided in Table 7.

TABLE 7

| FeNB thickness in FeTaN (50 nm)/FeNB/Glass (nm) | 0.5 GHz |              | 1 GHz  |              | 1.5 GHz |              | $f_r$ | Snoek product ( $\times 10^{12}$ ) |
|-------------------------------------------------|---------|--------------|--------|--------------|---------|--------------|-------|------------------------------------|
|                                                 | $\mu'$  | $\tan\delta$ | $\mu'$ | $\tan\delta$ | $\mu'$  | $\tan\delta$ | (GHz) |                                    |
| 15                                              | 985     | 0.52         | 1716   | 0.18         | 2850    | 0.54         | 1.90  | 1.87                               |
| 20                                              | 1386    | 0.18         | 1602   | 0.12         | 2680    | 0.51         | 1.87  | 2.59                               |
| 22                                              | 1416    | 0.27         | 1796   | 0.16         | 2351    | 0.47         | 1.83  | 2.59                               |

Example 5: FeNB/FeN/FeNB/Glass Tri-Layered Structure Parameters for RF Magnetron Sputtering

RF Power=80 to 120 W

Deposition pressure=0.3 to 0.6 pascals (Pa)

Distance between target and substrate=8 centimeters (cm)

Working gas: Ar (99.5%); Reaction gas: Nitrogen (99.0%)

Target:

Iron (99.5%), 2-inch disk

2 pieces of boron (99.5%) chip with  $5 \times 5 \text{ mm}^2$

1 piece for tantalum (99.99%) ( $5 \times 5 \text{ mm}^2$ )

Deposition time: 5 to 30 minutes

Deposition temperature: ambient

Substrate: Optical glass

Resistivity of FeNB/FeN/FeNB Structure

With reference to FIG. 18, the effective resistivity of a tri-layer film was measured by the V.D. Pauw method with four probes. The resistivity increased from 291 to 485  $\mu\Omega m$  for the total thickness of the tri-layer film from 55 to 125 nm. Details of film thickness and resistivity for  $Fe_{72}N_{18}B_{10}/Fe_{82}N_{18}/Fe_{72}N_{18}B_{10}$  tri-layer films are provided in Table 8.

TABLE 8

| Top layer FeNB (nm) | Middle layer FeN (nm) | Bottom layer FeNB (nm) | Total thickness (nm) | Resistivity ( $\mu\Omega m$ ) |
|---------------------|-----------------------|------------------------|----------------------|-------------------------------|
| 15                  | 20                    | 20                     | 55                   | 291                           |
| 15                  | 30                    | 30                     | 75                   | 351                           |
| 15                  | 35                    | 35                     | 85                   | 386                           |
| 20                  | 50                    | 25                     | 95                   | 455                           |
| 25                  | 50                    | 50                     | 125                  | 485                           |

Magnetic Permeability for FeNB/FeN/FeNB/Glass Structure

With reference to FIG. 19, the thickness of 50 nm for the FeN middle layer was fixed and the thicknesses of the top and bottom FeNB layer were changed. FIG. 19 shows  $\mu''$  (solid lines) and  $\mu''$  (dashed lines) for varying thicknesses of the top and bottom FeNB films in nm as indicated on the figure. The increased magnetic permeability (at 0.5 GHz)

and Snoek product were 995 and 2.16 for the FeNB(20 nm)/FeN(50 nm)/FeNB(25 nm) structures, respectively. Magnetic permeability of the FeNB(20 nm)/FeN(50 nm)/FeNB(25 nm) structure was about 50% higher than the FeNB(25 nm)/FeTaN(50 nm)/FeNB(25 nm) structure. A summary of magnetic spectrum measurements for  $Fe_{72}N_{18}B_{10}/Fe_{82}N_{18}/Fe_{72}N_{18}B_{10}$  tri-layer films is shown in Table 9. The last row includes details of the reference

TABLE 9

| Top layer    |              | FeNB<br>(nm) | Middle layer<br>FeN (nm) | Bottom layer |              | $\mu'$ at 0.5 GHz | $\mu'$ at 1.0 GHz | $\mu'$ at 1.5 GHz | $f_r$ | Snoek product<br>( $\times 10^{12}$ ) |
|--------------|--------------|--------------|--------------------------|--------------|--------------|-------------------|-------------------|-------------------|-------|---------------------------------------|
| FeNB<br>(nm) | FeNB<br>(nm) |              |                          | $\mu'$       | $\tan\delta$ | $\mu'$            | $\tan\delta$      | $\mu'$            | (GHz) |                                       |
| 20           | 50           | 25           | 995                      | 0.28         | 1339         | 0.27              | 1478              | 0.58              | 2.17  | 2.16                                  |
| 25           | 50           | 25           | 773                      | 0.33         | 1096         | 0.25              | 1444              | 0.53              | 2.21  | 1.71                                  |
| 25           | 50           | 50           | 530                      | 0.43         | 559          | 0.31              | 692               | 0.46              | 2.25  | 1.19                                  |
| 25           | 50 (FeTaN)   | 25           | 382                      | 0.41         | 457          | 0.16              | 464               | 0.96              | 1.79  | 0.68                                  |

Example 6: FeNB/FeTaN/FeNB/Glass Tri-Layered Structure Parameters for RF Magnetron Sputtering

RF Power=80 to 120 W

Deposition pressure=0.3 to 0.6 pascals (Pa)

Distance between target and substrate=8 centimeters (cm)

Working gas: Ar (99.5%); Reaction gas: Nitrogen (99.0%)

Target:

Iron (99.5%), 2-inch disk

2 pieces of boron (99.5%) chip with  $2.5 \times 2.5$  mm<sup>2</sup>

1 piece for tantalum (99.99%) (5×5 mm<sup>2</sup>)

GHz) and Snoek product were 545 and 1.14 for the FeNB(20 nm)/FeTaN(25 nm)/FeNB(25 nm) structures, respectively.

15 The magnetic permeability of the FeNB(20 nm)/FeTaN(25 nm)/FeNB(25 nm) structure was about 45% lower than that of the FeNB(20 nm)/FeN(50 nm)/FeNB(25 nm) structure (i.e., 995). A summary of magnetic spectrum measurements for  $\text{Fe}_{72}\text{N}_{18}\text{B}_{10}/\text{Fe}_{72}\text{TaN}_{18}\text{N}_{10}/\text{Fe}_{72}\text{N}_{18}\text{B}_{10}$  tri-layer films is provided in Table 11. The last row includes details of the reference sample.

TABLE 11

| Top layer |          | FeNB<br>(nm) | Middle layer<br>FeN (nm) | Bottom layer |        | $\mu'$ at 0.5 GHz | $\mu'$ at 1.0 GHz | $\mu'$ at 1.5 GHz | $f_r$ | Snoek product<br>( $\times 10^{12}$ ) |
|-----------|----------|--------------|--------------------------|--------------|--------|-------------------|-------------------|-------------------|-------|---------------------------------------|
| (nm)      | FeN (nm) |              |                          | FeNB (nm)    | $\mu'$ | $\tan\delta$      | $\mu'$            | $\tan\delta$      | (GHz) |                                       |
| 20        | 25       | 25           | 545                      | 0.31         | 504    | 0.11              | 712               | 0.35              | 2.09  | 1.14                                  |
| 25        | 25       | 25           | 511                      | 0.41         | 599    | 0.07              | 747               | 0.49              | 2.08  | 1.06                                  |
| 20        | 50       | 25           | 319                      | 0.62         | 429    | 0.23              | 425               | 0.83              | 1.86  | 0.59                                  |
| 25        | 50       | 25           | 382                      | 0.41         | 457    | 0.16              | 464               | 0.96              | 1.79  | 0.68                                  |
| 25        | 50       | 50           | 292                      | 0.02         | 397    | 0.04              | 382               | 0.91              | 1.76  | 0.52                                  |
| 20*       | 50 (FeN) | 25           | 995                      | 0.28         | 1366   | 0.27              | 1478              | 0.58              | 2.17  | 2.16                                  |

\*Reference example

35

Deposition time: 5 to 30 minutes

Deposition temperature: ambient

Substrate: Optical glass

Resistivity of FeNB/FeTaN/FeNB Structure

With reference to FIG. 20, the effective resistivity increased with an increase of total thickness of the tri-layer FeNB/FeTaN/FeNB film. The effective resistivity increased from 391 to 496  $\mu\Omega\text{m}$  for the total thickness from 70 to 125 nm. The effective resistivity of the FeNB/FeTaN/FeNB film was about 5% higher than that of the FeNB/FeN/FeNB film. Details of film thickness and resistivity for the  $\text{Fe}_{72}\text{N}_{18}\text{B}_{10}/\text{Fe}_{83}\text{Ta}_{6}\text{N}_{11}/\text{Fe}_{72}\text{N}_{18}\text{B}_{10}$  tri-layer structure are provided in Table 10.

40 RF Power=80 to 120 W

Deposition pressure=0.3 to 0.6 pascals (Pa)

Distance between target and substrate=8 centimeters (cm)

Working gas: Ar (99.5%); Reaction gas: Nitrogen (99.0%)

Target:

45 Iron (99.5%), 2-inch disk

2 pieces of boron (99.5%) chip with  $2.5 \times 2.5$  mm<sup>2</sup>

1 piece for tantalum (99.99%) (5×5 mm<sup>2</sup>)

Deposition time: 5 to 30 minutes

Deposition temperature: ambient

Substrate: Optical glass

Magnetic Permeability for FeN/TaN/Glass Structure

With reference to FIG. 22, a non-magnetic TaN film was a seed layer for the deposition of a 50 nm FeN film. FIG. 22 shows  $\mu'$  (solid lines) and  $\mu''$  (dashed lines) for varying thicknesses of the TaN films in nm as indicated on the figure.

55 The thickness of non-magnetic TaN seed layer varied from 15 to 30 nm. The increased magnetic permeability and Snoek product were 716 at 0.5 GHz and 1.53 when the thickness of TaN layer was about 20 nm. The magnetic permeability of the FeN(50 nm)/TaN(20 nm)/Glass structure was about 20% lower than that of the FeN(50 nm)/FeTaN(10 nm)/Glass structure (i.e., 892).

60 The magnetic seed layer resulted in frequency permeability higher than that of the non-magnetic seed layer (e.g., TaN). A summary of magnetic spectrum measurements for  $\text{Fe}_{82}\text{N}_{18}/\text{Ta}_{88}\text{N}_{12}$  bilayer films is provided in Table 12. The last row includes details of the reference sample.

TABLE 10

| Top layer<br>FeNB (nm) | Middle layer<br>FeTaN (nm) | Bottom layer<br>FeNB (nm) | Total thickness<br>(nm) | Resistivity<br>( $\mu\Omega\text{m}$ ) |
|------------------------|----------------------------|---------------------------|-------------------------|----------------------------------------|
| 20                     | 25                         | 25                        | 70                      | 396                                    |
| 20                     | 50                         | 25                        | 95                      | 437                                    |
| 25                     | 50                         | 25                        | 100                     | 468                                    |
| 25                     | 50                         | 50                        | 125                     | 496                                    |

Magnetic Permeability for FeNB/FeTaN/FeNB/Glass Structure

With reference to FIG. 21, the thickness of the FeNB and FeTaN layer varied from 20 nm to 50 nm. FIG. 21 shows  $\mu'$  (solid lines) and  $\mu''$  (dashed lines) for varying thicknesses of the top, middle, and bottom FeNB films in nm as indicated on the figure. The increased magnetic permeability (at 0.5

65 GHz) and Snoek product were 545 and 1.14 for the FeNB(20 nm)/FeTaN(25 nm)/FeNB(25 nm) structures, respectively. The magnetic permeability of the FeNB(20 nm)/FeTaN(25 nm)/FeNB(25 nm) structure was about 45% lower than that of the FeNB(20 nm)/FeN(50 nm)/FeNB(25 nm) structure (i.e., 995). A summary of magnetic spectrum measurements for  $\text{Fe}_{72}\text{N}_{18}\text{B}_{10}/\text{Fe}_{72}\text{TaN}_{18}\text{N}_{10}/\text{Fe}_{72}\text{N}_{18}\text{B}_{10}$  tri-layer films is provided in Table 11. The last row includes details of the reference sample.

TABLE 12

| Top layer | Bottom layer | $\mu'$ at 0.5 GHz |              | $\mu'$ at 1.0 GHz |              | $\mu'$ at 1.5 GHz |              | $f_r$ | Snoek product        |
|-----------|--------------|-------------------|--------------|-------------------|--------------|-------------------|--------------|-------|----------------------|
| FeN (nm)  | TaN (nm)     | $\mu'$            | $\tan\delta$ | $\mu'$            | $\tan\delta$ | $\mu'$            | $\tan\delta$ | (GHz) | ( $\times 10^{12}$ ) |
| 50        | 15           | 507               | 0.22         | 558               | 0.05         | 1220              | 0.17         | 2.12  | 1.07                 |
| 50        | 20           | 716               | 0.20         | 901               | 0.14         | 1939              | 0.17         | 2.13  | 1.53                 |
| 50        | 25           | 646               | 0.34         | 778               | 0.05         | 1494              | 0.15         | 2.16  | 1.39                 |
| 50        | 30           | 478               | 0.04         | 786               | 0.01         | 1648              | 0.09         | 2.09  | 1.00                 |
| 50*       | 20 (FeTaN)   | 892               | 0.08         | 1145              | 0.13         | 1709              | 0.89         | 1.76  | 1.57                 |

\*Reference example

## Magnetic Permeability for FeNB/TaN/Glass Structure

With reference to FIG. 23, the thickness of non-magnetic TaN seed layer varied from 10 nm to 25 nm. FIG. 23 shows  $\mu'$  (solid lines) and  $\mu''$  (dashed lines) for varying thicknesses of the TaN films in nm as indicated on the figure. The increased magnetic permeability and Snoek product were 937 at 0.5 GHz and 1.76 when the thickness of TaN seed layer was about 20 nm. The magnetic permeability of the FeN(50 nm)/TaN(20 nm)/Glass structure was about 32% lower than that of the FeNB(50 nm)/FeTaN(20 nm)/Glass structure (i.e., 1386). The magnetic permeability of the FeNB(50 nm)/TaN(20 nm)/Glass structure was about 24% higher than that of the FeN(50 nm)/TaN(20 nm)/Glass structure (i.e., 716). The magnetic seed layer demonstrated higher permeability than that of the non-magnetic seed layer. A summary of magnetic spectrum measurements for  $\text{Fe}_{72}\text{N}_{18}\text{B}_{10}/\text{TaN}_{88}\text{N}_{12}$  bilayer films is provided in Table 12. The last two rows include details of the reference samples.

TABLE 12

| Top layer | Bottom layer | $\mu'$ at 0.5 GHz |              | $\mu'$ at 1.0 GHz |              | $\mu'$ at 1.5 GHz |              | $f_r$ | Snoek product        |
|-----------|--------------|-------------------|--------------|-------------------|--------------|-------------------|--------------|-------|----------------------|
| FeN (nm)  | TaN (nm)     | $\mu'$            | $\tan\delta$ | $\mu'$            | $\tan\delta$ | $\mu'$            | $\tan\delta$ | (GHz) | ( $\times 10^{12}$ ) |
| 10        | 10           | 821               | 0.58         | 941               | 0.09         | 1598              | 0.20         | 2.01  | 1.65                 |
| 15        | 15           | 866               | 0.11         | 1043              | 0.12         | 2004              | 0.33         | 1.87  | 1.23                 |
| 20        | 20           | 937               | 0.17         | 1065              | 0.01         | 1827              | 0.32         | 1.88  | 1.76                 |
| 25        | 25           | 708               | 0.43         | 862               | 0.13         | 1378              | 0.16         | 2.06  | 1.46                 |
| 50*       | 20 (FeTaN)   | 1386              | 0.15         | 1581              | 0.13         | 2740              | 0.17         | 1.87  | 2.59                 |
| 50 (FeN)* | 20           | 716               | 0.20         | 901               | 0.14         | 1939              | 0.17         | 2.13  | 1.53                 |

\*Reference example

## Magnetic Permeability for FeTaN/TaN/Glass Structure

With reference to FIG. 24, the thickness of magnetic top FeTaN layer was fixed at 50 nm. FIG. 24 shows  $\mu'$  (solid lines) and  $\mu''$  (dashed lines) for varying thicknesses of the TaN films in nm as indicated on the figure. The thickness of non-magnetic TaN layer varied from 10 nm to 25 nm. The increased magnetic permeability and Snoek product was 832 at 0.5 GHz and 1.63 when the thickness of TaN layer was about 20 nm. The magnetic permeability of the FeTaN(50

nm)/TaN(20 nm)/Glass structure was about 38% lower than of the FeTaN(50 nm)/FeNB(20 nm)/Glass structure (i.e., 1386). The magnetic permeability of the FeTaN(50 nm)/TaN(20 nm)/Glass structure was about 14% higher than that of the FeN(50 nm)/TaN(20 nm)/Glass structure (i.e., 716). A summary of magnetic spectrum measurements for  $\text{Fe}_{83}\text{Ta}_6\text{N}_{11}/\text{TaN}_{88}\text{N}_{12}$  bilayer films is provided in Table 13. The last row includes details of the reference sample. The last two rows include details of the reference samples.

TABLE 13

| Top layer | Bottom layer | $\mu'$ at 0.5 GHz |              | $\mu'$ at 1.0 GHz |              | $\mu'$ at 1.5 GHz |              | $f_r$ | Snoek product        |
|-----------|--------------|-------------------|--------------|-------------------|--------------|-------------------|--------------|-------|----------------------|
| FeN (nm)  | TaN (nm)     | $\mu'$            | $\tan\delta$ | $\mu'$            | $\tan\delta$ | $\mu'$            | $\tan\delta$ | (GHz) | ( $\times 10^{12}$ ) |
| 10        | 10           | 669               | 0.68         | 911               | 0.18         | 1538              | 0.29         | 2.03  | 1.36                 |
| 15        | 15           | 714               | 0.49         | 1029              | 0.10         | 1814              | 0.25         | 1.99  | 1.42                 |
| 20        | 20           | 832               | 0.38         | 975               | 0.15         | 1697              | 0.29         | 1.96  | 1.63                 |
| 25        | 25           | 807               | 0.30         | 906               | 0.28         | 984               | 0.89         | 1.83  | 1.48                 |
| 50        | 20 (FeNB)    | 1386              | 0.20         | 1581              | 0.14         | 2740              | 0.17         | 1.87  | 2.59                 |
| 20 (FeN)  | 20           | 716               | 0.17         | 901               | 0.01         | 1939              | 0.32         | 2.13  | 1.53                 |

Example 8: Magnetic Permeability and Snoek Product Diagram of the FeN-Based or FeTaN-Based Multi-Layered Structure

Magnetic Permeability (at 0.5 GHz) and Snoek Product Diagram of FeN-Based Structure

With reference to FIG. 25, the magnetic permeability diagram at 0.5 GHz of the FeN-based film are provided for the single layer film, double layers film and triple layer structure. The increased magnetic permeability about 1800 was observed in the double-layered film with the 20~25 nm FeNB seed layer.

With reference to FIG. 26, the Snoek product diagram of the FeN-based film are provided for the single layer film, double layers film and triple layers film. The increased Snoek product about  $2.0\text{--}3.5 \times 10^{12}$  was observed in the double-layered film with the 20~25 nm FeNB seed layer.

Magnetic Permeability (at 0.5 GHz) and Snoek Product Diagram of FeTaN-Based Structure

With reference to FIG. 27, the magnetic permeability diagram of the FeTaN-based film is provided for the single layer film, double layers film and triple layers film. The increased magnetic permeability about 1300 was observed in the double-layered film with the 20~25 nm FeNB seed layer.

With reference to FIG. 28, the Snoek product diagram of the FeTaN-based film are provided for the single layer film, bi-layer film and triple-layer structure. The increased Snoek product about  $2.0 \times 10^{12}$  was observed in the double-layered film with the 20~25 nm FeTaN or FeNB seed layer.

Set forth below are some aspects of the multilayer magnetic film, articles comprising the same, and methods of making the same.

Aspect 1: A multilayer magnetic film, comprising: a substrate; a first magnetic layer disposed on the substrate, wherein the first magnetic layer comprises  $\text{Fe}_{(50\text{--}80)}\text{N}_{(10\text{--}20)}\text{B}_{(1\text{--}20)}\text{M}_{(0\text{--}10)}$ , wherein M is Si, Ta, Zr, Ti, Co, or a combination thereof; and a second magnetic layer disposed on the first magnetic layer, wherein the second magnetic layer comprises  $\text{Fe}_{(50\text{--}90)}\text{N}_{(10\text{--}50)}$  or  $\text{Fe}_{(60\text{--}90)}\text{N}_{(1\text{--}10)}\text{Ta}_{(5\text{--}30)}$ ; wherein the multilayer magnetic film has, over a frequency range of 50 MHz to 10 GHz, preferably over a frequency range of 100 MHz to 5 GHz, more preferably over a frequency range of 1 to 5 GHz, a magnetic permeability of greater than or equal to 1800, preferably greater than 2000, more preferably greater than 3000, or 1800 to 5000 over a selected frequency band in the frequency range, preferably over a frequency band of 1 to 10 GHz; a magnetic loss tangent of less than or equal to 0.3, preferably less than or equal to 0.1, or 0.01 to 0.3 over a selected frequency band in the frequency range, preferably over a frequency band of 1 to 10 GHz; and a cutoff frequency of greater than or equal to 1 GHz, greater than or equal to 1 GHz, or greater than or equal to 2 GHz, preferably greater than or equal to 5 GHz, or 1 to 8 GHz.

Aspect 2: The multilayer magnetic film of Aspect 1, wherein the substrate comprises a glass, polymer, or ceramic, preferably a ceramic.

Aspect 3: The multilayer magnetic film of any one or more of the preceding Aspects, wherein the first magnetic layer has a thickness of 10 to 100 nanometers, and the second magnetic layer has a thickness of 10 to 400 nanometers.

Aspect 4: The multilayer magnetic film of any one or more of the preceding Aspects, further comprising: an additional first layer comprising  $\text{Fe}_{(50\text{--}80)}\text{N}_{(10\text{--}20)}\text{B}_{(1\text{--}20)}$  disposed on the second layer; and an additional second mag-

netic layer comprising  $\text{Fe}_{(50\text{--}90)}\text{N}_{(10\text{--}50)}$  or  $\text{Fe}_{(60\text{--}90)}\text{N}_{(1\text{--}10)}\text{Ta}_{(5\text{--}30)}$  disposed on the additional first magnetic layer.

Aspect 5: The multilayer magnetic film of Aspect 4, comprising further additional first and second magnetic layers disposed on the additional second magnetic layer in alternation.

Aspect 6: The multilayer magnetic film of any one or more of Aspects 4 to 5, wherein the first magnetic layer and the second magnetic layer have a total thickness of 20 to 500 nanometers.

Aspect 7: An article comprising the multilayer film of any one or more of Aspects 1 to 6, preferably wherein the article is a filter, transformer, inductor, antenna, electronic integrated circuit chip, or electromagnetic shielding device.

Aspect 8: The article of Aspect 7, wherein the article is a component of an electronic device, preferably a mobile phone, a desktop computer, a laptop computer, a notebook computer, a wireless or LAN network, a power supply, an amplifier, a voltage-controlled oscillator, a shrink power converter, more preferably an integrated electronic device.

Aspect 9: A method of forming the multilayer magnetic film of any one or more of Aspects 1 to 6, the method comprising: depositing the first magnetic layer onto a side of the substrate; and depositing the second magnetic layer onto 25 a side of the first magnetic layer opposite to the substrate.

Aspect 10: The method of Aspect 9, wherein the depositing comprises rf/DC sputtering, electron beam deposition, or a combination thereof.

Aspect 11: The method of Aspect 10, further comprising 30 depositing an additional first layer on a side of the second layer opposite the first layer.

Aspect 12: The method of Aspect 11, further comprising depositing an additional second layer on a side of the additional first layer opposite the second layer.

Aspect 13: The method of any one or more of Aspects 9 to 12, comprising adjusting the thickness of each layer to 35 adjust the magnetic loss tangent of the multilayer magnetic film, the magnetic anisotropy of the magnetic multilayer film, or both.

Aspect 14: A multilayer magnetic film made by the method of any one or more of Aspects 9 to 13.

“Film” as used herein includes planar layers, sheets, and the like as well as other three-dimensional non-planar forms. A layer can further be macroscopically continuous or non-continuous. As used herein, “a,” “an,” “the,” and “at least one” do not denote a limitation of quantity, and are intended to cover both the singular and plural, unless the context clearly indicates otherwise. For example, “an element” has the same meaning as “at least one element,” unless the context clearly indicates otherwise. “Or” means “and/or.” Ranges disclosed herein are inclusive of the recited endpoint and are independently combinable. “Combination” is inclusive of blends, mixtures, alloys, reaction products, and the like. Also, “combination thereof” means that the list is 50 inclusive of each element individually, as well as combinations of two or more elements of the list, and combinations of at least one element of the list with like elements not named. The terms “first,” “second,” and so forth, herein do not denote any order, quantity, or importance, but rather are used to distinguish one element from another. While certain combinations of features have been described herein, it will be appreciated that these certain combinations are for illustration purposes only and that any combination of any of these features can be employed, explicitly or equivalently, either individually or in combination with any other of the features disclosed herein, in any combination, and all in accordance with an embodiment. Any and all such combi-

55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8

## 17

nations are contemplated herein and are considered within the scope of the disclosure. Unless otherwise stated, the test standards are the latest as of the date of filing.

The endpoints of all ranges directed to the same component or property are inclusive of the endpoints, are independently combinable, and include all intermediate points and ranges. For example, ranges of "up to 25, or 5 to 20" is inclusive of the endpoints and all intermediate values of the ranges of "5 to 25" such as 10 to 23, etc.

Unless defined otherwise, technical and scientific terms used herein have the same meaning as is commonly understood by one of skill in the art to which this invention belongs. All cited patents, patent applications, and other references are incorporated herein by reference in their entirety. However, if a term in the present application contradicts or conflicts with a term in the incorporated reference, the term from the present application takes precedence over the conflicting term from the incorporated reference.

While the disclosure has been described with reference to exemplary embodiments, it will be understood by those skilled in the art that various changes can be made, and equivalents can be substituted for elements thereof without departing from the scope of this disclosure. In addition, many modifications can be made to adapt a particular situation or material to the teachings without departing from the essential scope thereof. Therefore, it is intended that the disclosure not be limited to the particular embodiment disclosed as the best or only mode contemplated for carrying out this disclosure, but that the disclosure will include all embodiments falling within the scope of the appended claims. Also, in the drawings and the description, there have been disclosed exemplary embodiments and, although specific terms can have been employed, they are unless otherwise stated used in a generic and descriptive sense only and not for purposes of limitation.

What is claimed is:

1. A multilayer magnetic film, comprising:  
a substrate;  
a first magnetic layer disposed on the substrate, wherein  
the first magnetic layer comprises  $Fe_{(50-80)}N_{(10-20)}$   
 $B_{(1-20)}M_{(0-10)}$ , wherein M is Si, Ta, Zr, Ti, Co, or a  
combination thereof; and  
a second magnetic layer disposed on the first magnetic  
layer, wherein the second magnetic layer comprises  
 $Fe_{(50-90)}N_{(10-50)}$  or  $Fe_{(60-90)}N_{(1-10)}Ta_{(5-30)}$ ;  
wherein the multilayer magnetic film has, over a  
frequency range of 50 MHz to 10 GHz,

## 18

a magnetic permeability of greater than or equal to 1800 over a selected frequency band in the frequency range;

5 a magnetic loss tangent of less than or equal to 0.3 over a selected frequency band in the frequency range; and

a cutoff frequency of greater than or equal to 1 GHz.

2. The multilayer magnetic film of claim 1, wherein the substrate comprises a glass, polymer, or ceramic.

10 3. The multilayer magnetic film of claim 1, wherein the first magnetic layer has a thickness of 10 to 100 nanometers, and  
the second magnetic layer has a thickness of 10 to 400 nanometers.

15 4. The multilayer magnetic film of claim 1, further comprising:

an additional first layer comprising  $Fe_{(50-80)}N_{(10-20)}B_{(1-20)}$   
disposed on the second layer; and

20 an additional second magnetic layer comprising  $Fe_{(50-90)}N_{(10-50)}$  or  $Fe_{(60-90)}N_{(1-10)}Ta_{(5-30)}$  disposed on the additional first magnetic layer.

25 5. The multilayer magnetic film of claim 4, comprising further additional first and second magnetic layers disposed on the additional second magnetic layer in alternation.

6. The multilayer magnetic film of claim 4, wherein the first magnetic layer and the second magnetic layer have a total thickness of 20 to 500 nanometers.

7. An article comprising the multilayer film of claim 1.

8. The article of claim 7, wherein the article is a component of an electronic device.

30 9. A method of forming the multilayer magnetic film of claim 1, the method comprising:

depositing the first magnetic layer onto a side of the substrate; and

depositing the second magnetic layer onto a side of the first magnetic layer opposite to the substrate.

10. The method of claim 9, wherein the depositing comprises rf/DC sputtering, electron beam deposition, or a combination thereof.

11. The method of claim 10, further comprising depositing an additional first layer on a side of the second layer opposite the first layer.

12. The method of claim 11, further comprising depositing an additional second layer on a side of the additional first layer opposite the second layer.

13. The method of claim 9, comprising adjusting the thickness of each layer to adjust the magnetic loss tangent of the multilayer magnetic film, the magnetic anisotropy of the magnetic multilayer film, or both.

\* \* \* \* \*